# EUROPEAN PATENT SPECIFICATION

(11) **EP 3 872 212 B1**
(45) Date of publication and mention of the grant of the patent: **03.09.2025**
(21) Application number: 19875923.5
(22) Date of filing: 25.10.2019
(51) Int. Cl.: C22C 38/38, C22C 38/20, C22C 38/02, C22C 38/06, C22C 38/32, C21D 9/46, C21D 8/02, C21D 6/00, C21D 1/02

(54) **CRYOGENIC AUSTENITIC HIGH-MANGANESE STEEL HAVING EXCELLENT CORROSION RESISTANCE, AND MANUFACTURING METHOD THEREFOR**
KRYOGENER AUSTENITISCHER HOCHMANGANSTAHL MIT AUSGEZEICHNETER KORROSIONSBESTÄNDIGKEIT UND VERFAHREN ZU SEINER HERSTELLUNG
ACIER AUSTÉNITIQUE CRYOGÉNIQUE À HAUTE TENEUR EN MANGANÈSE AYANT UNE EXCELLENTE RÉSISTANCE À LA CORROSION ET PROCÉDÉ DE FABRICATION ASSOCIÉ

(30) Priority: 25.10.2018 KR 20180128505
(43) Date of publication of application: 01.09.2021
(73) Proprietor: POSCO Co., Ltd, Pohang-si, Gyeongsangbuk-do 37859 (KR)
(72) Inventor: LEE, Un-Hae, Gwangyang-si, Jeollanam-do 57807 (KR); LEE, Dong-Ho, Gwangyang-si, Jeollanam-do 57807 (KR); KANG, Sang-Deok, Gwangyang-si, Jeollanam-do 57807 (KR); KIM, Sung-Kyu, Gwangyang-si, Jeollanam-do 57807 (KR)
(74) Representative: Meissner Bolte Partnerschaft mbB
(86) International application number: PCT/KR2019/014197
(87) International publication number: WO 2020/085864

(56) References cited:
- WO-A1-2017/111510
- CN-A- 106 222 554
- CN-A- 107 177 786
- CN-A- 107 620 010
- JP-A- 2007 126 715
- JP-A- 2007 126 715
- JP-A- 2016 196 703
- JP-A- S5 623 259
- KR-A- 20160 078 664
- KR-A- 20180 072 967
- KR-A- 20180 074 450
- KR-A- 20180 074 450

## Description

### [Technical Field]

The present invention relates to an austenitic high-manganese steel material and a method of manufacturing the same, and more particularly, an austenitic high-manganese steel material having excellent cryogenic toughness and excellent corrosion resistance, and a method of manufacturing the same.

### [Background Art]

As regulations on environmental pollution have been strengthened, and depletion of petroleum energy has been expected, demand for eco-friendly energy such as LNG and LPG has increased as alternative energy, and interest in development of use technology has increased. As demand for low-polluting fuels such as LNG and LPG, which may be transported in a low-temperature liquid state, has increased, development of materials for low-temperature structures for storage and transportation thereof has been actively conducted. A material for a low-temperature structure may require mechanical properties such as low-temperature strength and toughness, and the most representative material for a low-temperature structure may include 9% Ni steel material or 304 stainless steel material.

9% Ni steel material may exhibit excellent properties in terms of weldability and economic efficiency, but may have a level of corrosion resistance similar to that of a general carbon steel material, and therefore, particularly, application thereof in an environment accompanied with deformation and corrosion may not be preferable. Also, while a 304 stainless steel material has excellent corrosion resistance properties; there may be technical difficulties in terms of securing economic efficiency and low-temperature properties. Therefore, it may be urgent to develop a material having excellent low-temperature properties and excellent corrosion resistance.

CN106222554 A discloses an economic ultra-low temperature high Mn austenitic steel, having excellent low-temperature toughness.

### [Prior Art Document]

(Reference 1) Korean Laid-Open Patent Publication No. 10-2015-0075324 (publicized on July 3, 2015)

(Reference 2) CN106222554 A

### [Disclosure]

### [Technical Problem]

The present invention provides a

cryogenic austenitic high-manganese steel material having excellent corrosion resistance and a method of manufacturing the same.

### [Technical Solution]

The invention is defined in the appended claims.

A grain size of austenite may be 5-150 µm.

various features of the present invention and advantages and effects thereof will be understood in greater detail with reference to the specific embodiments as below.

### [Advantageous Effects]

According to the present invention, a cryogenic austenitic high-manganese steel material having excellent cryogenic toughness and having excellent corrosion resistance, and a method of manufacturing the same are provided.

### [Best Mode for Invention]

The present disclosure relates to a cryogenic austenitic high-manganese steel material having excellent corrosion resistance and a method of manufacturing the same, and hereinafter, preferable embodiments of the present disclosure will be described. Embodiments of the present disclosure may be modified in various forms, and the scope of the present disclosure should not be construed as being limited to the embodiments described below. The embodiments are provided to further describe the present disclosure to a person skilled in the art to which the present disclosure pertains.

Hereinafter, a steel composition in the present disclosure will be described in greater detail. Hereinafter, "%" indicating a content of each element may be based on weight unless otherwise indicated.

The cryogenic austenitic high-manganese steel material having excellent corrosion resistance according to an aspect of the present disclosure includes 0.2-0.5% of C, 23-28% of Mn, 0.05-0.5% of Si, 0.03% or less of P, 0.005% or less of S, 0.001-0.05% of Al, 3-4% of Cr, 0.3-1% of Cu, optionally 0.0005-0.01% of B, and a balance of Fe and inevitable impurities.

### Carbon (C): 0.2-0.5%

Carbon (C) is effective in stabilizing austenite in a steel material and securing strength by solid solution strengthening. Accordingly, in the present disclosure, a lower limit of the carbon (C) content is limited to 0.2% to secure low-temperature toughness and strength. In other words, when the carbon (C) content is less than 0.2%, austenite stability may be insufficient such that stable austenite may not be obtained at cryogenic temperature, and processing organic transformation into ε-martensite and α'-martensite may easily occur by external stress such that toughness and strength of the steel material may be reduced. When the carbon (C) content exceeds a certain range, toughness of the steel material may be rapidly deteriorated due to precipitation of carbides, and strength of the steel material may excessively increase such that workability of the steel material may significantly degrade. Thus, an upper limit of the carbon (C) content is limited to 0.5%. Therefore, the carbon (C) content in the present disclosure is 0.2-0.5%. A preferable carbon (C) content may be 0.3-0.5%, and a more preferable carbon (C) content may be 0.35-0.5%.

### Manganese (Mn): 23-28%

Manganese (Mn) is an important element which may stabilize austenite, and accordingly, in the present disclosure, a lower limit of the manganese (Mn) content is limited to 23% to obtain the effect as above. In other words, since 23% or more of manganese (Mn) is included in the present disclosure, stability of austenite may effective increase, such that the formation of ferrite, ε-martensite, and α'-martensite may be inhibited, thereby effectively securing low-temperature toughness of the steel material. When the manganese (Mn) content exceeds a certain level, the effect of increasing stability of austenite may be saturated, but manufacturing costs may greatly increase, and internal oxidation may excessively occur during hot-rolling, such that surface quality may be deteriorated. Thus, an upper limit of the manganese (Mn) content is limited to 28%. Accordingly, the manganese (Mn) content in the present disclosure is 23-28%, and a more preferable manganese (Mn) content may be 23-25%.

### Silicon (Si): 0.05-0.5%

Silicon (Si) is a deoxidizing agent as aluminum (Al) and may be inevitably added in a small amount. When silicon (Si) is excessively added, oxide may be formed on a grain boundary such that high-temperature ductility may be reduced, and cracks may be created such that surface quality may be deteriorated. Thus, an upper limit of the silicon (Si) content is limited to 0.5%. Since excessive costs may be required to reduce the silicon (Si) content in steel, a lower limit of the silicon (Si) content is limited to 0.05% in the present disclosure. Therefore, the silicon (Si) content in the present disclosure is 0.05-0.5%.

### Phosphorus (P): 0.03% or less

Phosphorus (P) may be easily segregated and may cause cracking during casting or may degrade weldability. Accordingly, in the present disclosure, an upper limit of the phosphorus (P) content is limited to 0.03% to prevent deterioration of castability and weldability. Also, in the present disclosure, a lower limit of the phosphorus (P) content may not be particularly limited, but may be limit to 0.001% in consideration of steel making burden.

### Sulfur (S): 0.005% or less

Sulfur (S) may cause a hot brittleness defect by forming inclusions. Accordingly, in the present disclosure, an upper limit of the sulfur (S) content is limited to 0.005% to inhibit hot brittleness. Also, in the present disclosure, a lower limit of the sulfur (S) content may not be particularly limited, but may be limited to 0.0005% in consideration of steel making burden.

### Aluminum (Al): 0.001-0.05%

Aluminum (Al) is a representative element added as a deoxidizer. Accordingly, in the present disclosure, a lower limit of the aluminum (Al) content is limited to 0.001%, and more preferably to 0.005% to obtain the effect as above. Aluminum (Al), however, may form precipitates by reacting with carbon (C) and nitrogen (N), and hot workability may be deteriorated by the precipitates. Thus, an upper limit of the aluminum (Al) content is limited to 0.05%. A more preferable upper limit of the aluminum (Al) content may be 0.045%.

### Chromium (Cr): 3-4%

Chromium (Cr) may stabilize austenite in a range of an appropriate amount such that chromium (Cr) may contribute to improving impact toughness at low temperature, and may be solid-solute in austenite and may increase strength of the steel material. Also, chromium may effectively contribute to improving corrosion resistance of the steel material. Therefore, in the present disclosure, 3% or more of chromium (Cr) is added to obtain the effect as above. However, chromium (Cr) may be a carbide-forming element and may form carbides on an austenite grain boundary, such that low-temperature impact toughness may be reduced. Thus, an upper limit of the chromium (Cr) content is limited to 4% in consideration of content relationship between carbon (C) and other elements added together. Accordingly, the chromium (Cr) content in the present disclosure is 3-4%, and a more preferable chromium (Cr) content may be 3-3.8%.

The cryogenic austenitic high-manganese steel material having excellent scale peelability according to an aspect of the present disclosure includes, by weight%, 0.3-1% of Cu, and optionally 0.0005-0.01% of B.

### Copper (Cu): 0.3-1%

Copper (Cu) may stabilize austenite together with manganese (Mn) and carbon (C), and may effectively contribute to improving low-temperature toughness of the steel material. Also, copper (Cu) may have an extremely low solubility in carbides and may be slowly diffused in austenite, such that copper (Cu) may be concentrated on an interfacial surface between austenite and carbide and may surround a nuclei of fine carbide, thereby effectively inhibiting formation and growth of carbides caused by additional diffusion of carbon (C). Thus, in the present disclosure, copper (Cu) is added to secure low-temperature toughness, and a lower limit of the copper (Cu) content is 0.3%. A more preferable lower limit of the copper (Cu) content may be 0.4%. When the copper (Cu) content exceeds 1%, hot workability of the steel material may be deteriorated, and in the present disclosure, an upper limit of the copper (Cu) content is limited to 1%. Thus, the copper (Cu) content in the present disclosure is 0.3-1% and a more preferable upper limit of the copper (Cu) content may be 0.7%.

### Boron (B): 0.0005-0.01%

Boron (B) may be a grain boundary strengthening element which may strengthen an austenite grain boundary, and by even adding boron (B) in a small amount, an austenite grain boundary may be strengthened such that high-temperature cracking sensitivity may be effectively reduced. To obtain the effect as above, in the present disclosure, 0.0005% or more of boron (B) is added. A preferable lower limit of the boron (B) content may be 0.001%, and a more preferable lower limit of the boron (B) content may be 0.002%. When the boron (B) content exceeds a certain range, segregation may occur on an austenite grain boundary such that high-temperature cracking sensitivity of the steel material may increase, and surface quality of the steel material may be degraded. Thus, in the present disclosure, an upper limit of the boron (B) content is limited to 0.01%. A preferable upper limit of the boron (B) content may be 0.008%, and a more preferable upper limit of the boron (B) content may be 0.006%.

The cryogenic austenitic high-manganese steel material having excellent scale peelability according to the present disclosure has a remainder of Fe and inevitable impurities in addition to the elements described above. In a general manufacturing process, inevitable impurities may be inevitably added from raw materials or an ambient environment, and thus, impurities may not be excluded. A person skilled in the art of a general manufacturing process may be aware of the impurities, and thus, the descriptions of the impurities may not be provided in the present disclosure.

The cryogenic austenitic high-manganese steel material having excellent corrosion resistance according to an aspect of the present disclosure may include 95 area% or more of austenite as a microstructure, thereby effectively securing cryogenic toughness of the steel material. An average grain size of austenite may be 5-150 µm. An average grain size of austenite implementable in the manufacturing process may be 5 µm or more, and when the average grain size increases significantly, strength of the steel material may be reduced. Thus, the grain size of austenite may be limited to 150 µm or less.

The cryogenic austenitic high-manganese steel material having excellent corrosion resistance according to an aspect of the present disclosure may include carbide and/or ε-martensite as a possible structure other than austenite. When a fraction of carbide and/or ε-martensite exceeds a certain level, toughness and ductility of the steel material may be rapidly deteriorated. Thus, in the present disclosure, the fraction of carbide and/or ε-martensite may be limited to 5 area% or less.

The cryogenic austenitic high-manganese steel material having excellent corrosion resistance according to an aspect of the present disclosure includes a Cr concentration section continuously formed in an area within 50 µm from a surface in a thickness direction of the steel material. The Cr concentration section refers to an area having a high Cr content as compared to the Cr content of the entire steel material.

The inventor of the present disclosure has conducted in-depth research on a Cr-added steel material in relation to a measure for improving corrosion resistance of a high manganese steel material, and as a result, it has been confirmed that, even when the same amount of Cr is added to the steel material, corrosion resistance properties may differ depending on the distribution of the Cr content in the Cr concentration section formed on the surface side of the steel material. In other words, in the case of Cr-added high manganese steel material, the Cr in steel may be concentrated in a surface layer of the steel material due to heating during the manufacturing process such that a Cr concentration section may be formed, and an aspect of Cr distribution in the Cr concentration section may be varied depending on heating conditions. Also, although it may be difficult to prove the exact mechanism, it has been indicated that, as for high manganese steel to which the same content of Cr is added, a steel material in which the Cr content in the Cr concentration section is uniformly distributed had further improved corrosion resistance properties as compared to a steel material in which a large amount of Cr is locally concentrated in the Cr concentration section. Therefore, the inventor of the present disclosure added Cr within an optimum range to secure corrosion resistance and low temperature properties of the steel material, and conducted an in-depth study on the surface layer Cr concentration conditions in which optimum corrosion resistance may be implemented even within the corresponding Cr content range, and completed the present disclosure.

The Cr concentration section in the present disclosure is formed in an area within 50 µm in the thickness direction from the surface of the steel material, and is continuously formed in the entire surface layer direction of the steel material. In other words, the Cr concentration section may include a case in which the Cr concentration section is formed directly below the surface of the steel material, and also a case in which the Cr concentration section is formed in contact with the surface of the steel material or is formed to form the surface of the steel material.

The Cr concentration section includes a high Cr concentration section in which Cr is concentrated in a relatively high concentration and a low Cr concentration section in which Cr is concentrated in a relatively low concentration. The high Cr concentration section refers to an area including Cr by more than 1.5 times the Cr content of the steel material, and the low Cr concentration section refers to an area including Cr by more than 1 time and 1.5 times or less the Cr content of the steel material. For example, in a steel material having the Cr content of 3.4% in the entire steel material, an area in which the Cr content is measured as 6% may be classified as the high Cr concentration section, and an area in which the Cr content is measured 4% may be classified as the low Cr concentration section. Also, since a heating process is essentially involved in the process of manufacturing the steel material, the surface layer of the steel material may exhibit a Cr content relatively higher than that of the entire steel material. Therefore, in the present disclosure, the Cr concentration section refers to an area including Cr by more than 1 times as compared to the Cr content of the steel material. The Cr concentration in the surface layer of steel material is measured with a scanning electron microscope (SEM). Also, the area fractions of the high Cr concentration section and the low Cr concentration section are calculated from the results of observation using a scanning electron microscope.

On the surface of the steel material, when Cr is locally concentrated in a partial area of the surface portion, a relatively low concentration of Cr may be distributed in the other area of the surface portion. Therefore, a corrosion resistance effect may be relatively lowered in an area other than the area in which Cr is locally concentrated, and thus, it is preferable to distribute Cr evenly in the surface layer of the steel material. In terms of securing corrosion resistance, the high Cr concentration section in the present disclosure is provided in a fraction of 30 area% or less (excluding 0%) relative to the entire area of the Cr concentration section, and may be provided in a fraction of 10 area% or less more preferably.

The cryogenic austenitic high-manganese steel material having excellent corrosion resistance according to the present disclosure has a yield strength of 400 MPa or more, a tensile strength of 800 MPa or more, and an elongation of 40% or more. Also, the cryogenic austenitic high-manganese steel material having excellent corrosion resistance according to the present disclosure has a Charpy impact toughness of 90J or more (based on a 10mm sample thickness) at -196°C, and corrosion loss of 80mg/cm² or less in a corrosion resistance test according to ISO9223. Accordingly, both excellent cryogenic properties and excellent corrosion resistance properties may be provided.

Hereinafter, the manufacturing method in the present disclosure will be described in greater detail.

A method of manufacturing a cryogenic austenitic high-manganese steel material having excellent corrosion resistance according to an aspect of the present disclosure includes reheating a slab including, by weight%, 0.2-0.5% of C, 23-28% of Mn, 0.05-0.5% of Si, 0.03% or less of P, 0.005% or less of S, 0.001-0.05% of Al, 3-4% of Cr, 0.3-1% of Cu, optionally 0.0005-0.01% of B, and a balance of Fe and inevitable impurities, in a temperature range of 1050-1300°C; hot-rolling the reheated slab at a finishing rolling temperature of 900-950°C, thereby providing an intermediate material; and cooling the intermediate material to a temperature range of 600°C or less at a cooling rate of 10-100°C/s, thereby providing a final material.

### Reheating slab

Since the slab provided in the manufacturing method in the present disclosure corresponds to the steel composition of the austenitic high-manganese steel material described above, the description of the steel composition of the slab is replaced with the description of the steel composition of the austenitic high-manganese steel material described above

The slab provided in the above-described steel composition is reheated in a temperature range of 1050-1300°C. When the reheating temperature is less than a certain range, there may be a problem in which an excessive rolling load may be applied during hot-rolling, or an alloy component may not be sufficiently solid solute. Therefore, in the present disclosure, a lower limit of the slab reheating temperature range is limited to 1050°C. When the reheating temperature exceeds a certain range, grains may excessively grow such that strength of the steel material may be deteriorated, or the reheating may be performed by exceeding a solidus temperature of the steel material such that hot-rolling properties of the steel material may be deteriorated. Thus, an upper limit of the reheating temperature range is limited to 1300°C.

### Hot-rolling

The hot-rolling process may include a rough-rolling process and a finishing rolling process, and the reheated slab may be hot-rolled and may be provided as an intermediate material. In this case, the finish hot-rolling is performed in a temperature range of 900-950°C. When the finishing hot-rolling temperature is excessively low, mechanical strength may increase, whereas low-temperature impact toughness may be deteriorated, and thus, in the present disclosure, the finishing hot-rolling temperature is limited to 900°C or higher. Also, when the finishing hot-rolling temperature is excessively high, low-temperature impact toughness may improve, whereas the local Cr concentration tendency of the surface layer portion of the steel material may increase, and thus, in the present disclosure, the finishing hot-rolling temperature is limited to 950°C in terms of securing corrosion resistance.

### Cooling

The hot-rolled intermediate material is cooled to a cooling stop temperature of 600°C or less at a cooling rate of 10-100°C/s. When the cooling rate is less than a certain range, a decrease in ductility of the steel material and deterioration of abrasion resistance may become problems due to carbides precipitated on a grain boundary during cooling, and thus, in the present disclosure, the rate of cooling the hot-rolled material is limited to 10°C/s or more. The higher the cooling rate is, the more advantageous the effect of inhibiting carbide precipitation may be, but in consideration of a situation in which it may be difficult to implement a cooling rate exceeding 100°C/s in general cooling in terms of characteristics of facility, an upper limit of the cooling rate is limited to 100°C/s in the present disclosure. Accelerated cooling may be applied to the cooling in the present disclosure.

Also, even when the intermediate material is cooled by applying a cooling rate of 10°C/s or more, when the cooling is stopped at a high temperature, it may be highly likely that carbides may be created and grown, and thus, in the present disclosure, the cooling stop temperature is limited to 600°C or less.

The austenitic high-manganese steel material manufactured as above includes a Cr concentration section continuously formed in an area within 50 µm from a surface in a thickness direction, the Cr concentration section includes a high Cr concentration section in which Cr is concentrated in a relatively high concentration and a low Cr concentration section in which Cr is concentrated in a relatively low concentration, and the high Cr concentration section is distributed in a fraction of 30 area% or less (excluding 0%) relative to an entire surface area of the Cr concentration section.

Also, the austenitic high-manganese steel material manufactured as above has a yield strength of 400 MPa or more, a tensile strength of 800 MPa or more, and an elongation of 40% or more, and the steel material has a Charpy impact toughness of 90J or more (based on a 10mm sample thickness) at -196°C, and corrosion loss of 80mg/cm² or less in a corrosion resistance test according to ISO9223.

### [Best Mode for Invention]

### (Embodiment)

A slab provided in the alloy composition as in Table 1 was prepared, and each sample was manufactured by applying the manufacturing process as in Table 2.

**[Table 1]**

| Clas | Alloy composition (weight%) | | | | | | | |
|---|---|---|---|---|---|---|---|---|
| sifi cati on | C | Si | Mn | Cr | P | S | Al | Cu |
| Stee l type 1 | 0.4 6 | 0.3 3 | 24. 0 | 3.4 2 | 0.01 3 | 0.00 2 | 0.02 4 | 0.5 0 |
| Stee l type 2 | 0.4 5 | 0.2 8 | 24. 1 | 3.2 1 | 0.01 4 | 0.00 1 | 0.02 4 | 0.4 3 |
| Stee l type 3 | 0.4 2 | 0.2 6 | 23. 9 | - | 0.01 8 | 0.00 2 | 0.02 8 | 0.3 8 |

**[Table 2]**

| Sample No. | Classif ication | Heating slab | | Hot-rolling | | Coolin g rate (°C/s) |
|---|---|---|---|---|---|---|
| | | Furnace tempera ture (°C) | Dischar ging Tempera ture (°C) | Finish rollin g temper ature (°C) | Final thickn ess (mm) | |
| 1 | Steel type 1 | 1218 | 1169 | 900 | 25 | 25 |
| 2 | Steel type 2 | 1225 | 1172 | 910 | 24 | 21 |
| 3 | Steel type 1 | 1218 | 1165 | 925 | 38 | 26 |
| 4 | Steel type 2 | 1225 | 1160 | 942 | 24 | 19 |
| 5 | Steel type 2 | 1225 | 1162 | 918 | 22 | 21 |
| 6 | Steel type 3 | 1220 | 1158 | 890 | 25 | 23 |
| 7 | Steel type 3 | 1221 | 1160 | 932 | 25 | 22 |
| 8 | Steel type 3 | 1220 | 1160 | 959 | 22 | 22 |
| 9 | Steel type 2 | 1211 | 1154 | 969 | 40 | 20 |
| 10 | Steel type 2 | 1215 | 1161 | 852 | 40 | 21 |

Tensile properties and impact toughness of each sample were evaluated, and the results thereof are listed in Table 3. Tensile properties of each sample were evaluated by conducting a test at room temperature according to ASTM A370, and impact toughness was measured at -196°C by processing into impact samples having a thickness of 10 mm according to the conditions of the same standard. Also, the Cr concentration section of the surface layer portion was observed using a scanning electron microscope (SEM) for each sample, and an area fraction of the high Cr concentration section relative to the surface area of the sample was calculated. Also, in accordance with the ISO9223 corrosion reduction test conditions, for each sample, a mild steel material standard sample and an each evaluation sample were exposed under wet conditions (50°C, 95%RH), corrosion was performed until the time point (takes 70 days) in which the corrosion amount of the mild steel material standard sample reach 1 year corrosion amount (52.5 mg/cm²) of atmospheric corrosion, and corrosion loss of the evaluation sample was analyzed.

**[Table 3]**

| Sample No. | Clas sifi cati on | Tensile properties | | | C direction Impact toughness @-(J, 196°C) | High Cr conce ntrat ion secti on Fract ion (area %) | Corros ion loss (mg/cm ²) |
|---|---|---|---|---|---|---|---|
| | | Yield streng th (MPa) | Tensil e streng th (MPa) | Elon gati on (%) | | | |
| 1 | Stee l type 1 | 485 | 868 | 57 | 105 | 6 | 55 |
| 2 | Stee l type 2 | 454 | 867 | 56 | 106 | 7 | 59 |
| 3 | Stee l type 1 | 483 | 872 | 59 | 108 | 11 | 62 |
| 4 | Stee l type 2 | 446 | 852 | 54 | 103 | 14 | 67 |
| 5 | Stee l type 2 | 471 | 878 | 57 | 98 | 13 | 65 |
| 6 | Stee l type 3 | 441 | 858 | 55 | 96 | - | 105 |
| 7 | Stee l type 3 | 425 | 851 | 56 | 101 | - | 112 |
| 8 | Stee l type 3 | 325 | 782 | 60 | 112 | - | 118 |
| 9 | Stee l type 2 | 351 | 792 | 66 | 125 | 37 | 91 |
| 10 | Stee l type 2 | 590 | 945 | 39 | 82 | 8 | 57 |

As indicated in Tables 1 to 3, it has been indicated that samples 1 to 5 satisfying the alloy composition and the process conditions of the present disclosure satisfied yield strength of 400 MPa or more, tensile strength of 800 MPa or more, elongation of 40% or more, and Charpy impact toughness (based on 10mm sample thickness) of 90J or more at -196°C, and that the fraction of high Cr concentration section satisfied 30 area% or less, such that corrosion loss in the corrosion test of ISO9223 was 80mg/cm² or less. Samples 6 to 10 which did not satisfy any one or more of the alloy composition or the process conditions of the present disclosure did not satisfy any one or more of the physical properties.

While the example embodiments have been illustrated and described above, it will be apparent to those skilled in the art that modifications and variations could be made without departing from the scope of the present disclosure as defined by the appended claims.

## Claims

1. A cryogenic austenitic high-manganese steel material having excellent corrosion resistance, comprising:
by weight%, 0.2-0.5% of C, 23-28% of Mn, 0.05-0.5% of Si, 0.03% or less of P, 0.005% or less of S, 0.001-0.05% of Al, 3-4% of Cr, 0.3-1% of Cu, optionally 0.0005-0.01%. of B, and a balance of Fe and inevitable impurities; and
a Cr concentration section continuously formed in an area within 50 µm from a surface in a thickness direction,
wherein the Cr concentration section includes a high Cr concentration section including Cr by more than 1.5 times the Cr contents of the steel material and a low Cr concentration section including Cr by more than 1 time and 1.5 times or less the Cr content of the steel material, and
wherein the high Cr concentration section is distributed in a fraction of 30 area% or less, excluding 0%, relative to an entire surface area of the Cr concentration section,
wherein a yield strength of the steel material measured by a tensile property test according to ASTM A370 is 400 MPa or more, a tensile strength of the steel material measured by a tensile property test according to ASTM A370 is 800 MPa or more, an elongation of the steel material measured by a tensile property test according to ASTM A370 is 40% or more, a Charpy impact toughness the steel material measured by an impact toughness property test according to ASTM A370 using a specimen having a thickness of 10mm sample thickness is 90J or more at -196°C, and a corrosion loss of the steel material measured as disclosed in the description by a corrosion resistance test according to ISO9223 of 80mg/cm² or less, and
wherein area fraction of the high Cr concentration section is calculated by observing a surface portions of the specimen using a scanning electron microscope.

2. The steel material of claim 1, wherein the high Cr concentration section is distributed in a fraction of 10 area% or less relative to an entire surface area of the Cr concentration section.

3. The steel material of claim 1, wherein a grain size of austenite is 5-150µm.

4. A method of manufacturing a cryogenic austenitic high-manganese steel material having excellent corrosion resistance of claim 1, the method comprising:
reheating a slab including, by weight%, 0.2-0.5% of C, 23-28% of Mn, 0.05-0.5% of Si, 0.03% or less of P, 0.005% or less of S, 0.001-0.05% of Al, 3-4% of Cr, 0.3-1% of Cu, optionally 0.0005-0.01% of B, and a balance of Fe and inevitable impurities, in a temperature range of 1050-1300°C;
hot-rolling the reheated slab at a finishing rolling temperature of 900-950°C, thereby providing an intermediate material; and
cooling the intermediate material to a temperature range of 600°C or less at a cooling rate of 10-100°C/s, thereby providing a final material.

## Patentansprüche

1. Kryogenes austenitisches Hochmanganstahlmaterial mit ausgezeichneter Korrosionsbeständigkeit, umfassend:
nach Gewichts-%, 0,2-0,5 % C, 23-28 % Mn, 0,05-0,5 % Si, 0,03 % oder weniger P, 0,005 % oder weniger S, 0,001-0,05 % Al, 3-4 % Cr, 0,3-1 % Cu, gegebenenfalls 0,0005-0,01 % B und einen Rest Fe und unvermeidbare Verunreinigungen; und
einen Cr-Konzentrationsteil, der kontinuierlich in einem Bereich innerhalb von 50 µm von einer Oberfläche in einer Dickenrichtung gebildet ist,
wobei der Cr-Konzentrationsteil einen hohen Cr-Konzentrationsteil, der Cr um mehr als das 1,5-Fache des Cr-Gehalts des Stahlmaterials beinhaltet, und einen geringen Cr-Konzentrationsteil, der Cr um mehr als das 1-Fache und das 1,5-Fache oder weniger des Cr-Gehalts des Stahlmaterials beinhaltet, beinhaltet und
wobei der hohe Cr-Konzentrationsteil in einem Anteil von 30 Flächen-% oder weniger, ausschließlich 0 %, relativ zu einem gesamten Oberflächenbereich des Cr-Konzentrationsteils verteilt ist,
wobei eine Streckgrenze des Stahlmaterials, gemessen durch einen Zugeigenschaftstest gemäß ASTM A370, 400 MPa oder mehr beträgt, eine Zugfestigkeit des Stahlmaterials, gemessen durch einen Zugeigenschaftstest gemäß ASTM A370, 800 MPa oder mehr beträgt, eine Ausdehnung des Stahlmaterials, gemessen durch einen Zugeigenschaftstest gemäß ASTM A370, 40 % oder mehr beträgt, eine Charpy-Schlagzähigkeit des Stahlmaterials, gemessen durch einen Schlagzähigkeitseigenschaftstest gemäß ASTM A370 unter Verwendung einer Probe, die eine Dicke von 10 mm Probendicke aufweist, 90 J oder mehr bei -196 °C aufweist und ein Korrosionsverlust des Stahlmaterials, gemessen gemäß der Offenbarung in der Beschreibung durch einen Korrosionsbeständigkeitstest gemäß ISO9223, 80 mg/cm² oder weniger beträgt, und
wobei der Flächenanteil des hohen Cr-Konzentrationsteils durch Beobachten eines Oberflächenabschnitts der Probe unter Verwendung eines Rasterelektronenmikroskops berechnet wird.

2. Stahlmaterial nach Anspruch 1, wobei der hohe Cr-Konzentrationsteil in einem Anteil von 10 Flächen-% oder weniger relativ zu einem gesamten Oberflächenbereich des Cr-Konzentrationsteils verteilt ist.

3. Stahlmaterial nach Anspruch 1, wobei eine Korngröße von Austenit 5-150 µm beträgt.

4. Verfahren zum Herstellen eines kryogenen austenitischen Hochmanganstahlmaterials mit ausgezeichneter Korrosionsbeständigkeit nach Anspruch 1, wobei das Verfahren Folgendes umfasst:
Aufwärmen einer Bramme, die, nach Gewichts-%, 0,2-0,5 % C, 23-28 % Mn, 0,05-0,5 % Si, 0,03 % oder weniger P, 0,005 % oder weniger S, 0,001-0,05 % Al, 3-4 % Cr, 0,3-1 % Cu, gegebenenfalls 0,0005-0,01 % B und einen Rest Fe und unvermeidbare Verunreinigungen beinhaltet, in einem Temperaturbereich von 1050-1300 °C;
Warmwalzen der aufgewärmten Bramme bei einer Fertigwalztemperatur von 900-950 °C, wodurch ein Zwischenmaterial bereitgestellt wird; und
Abkühlen des Zwischenmaterials auf einen Temperaturbereich von 600 °C oder weniger bei einer Abkühlungsgeschwindigkeit von 10-100 °C/s, wodurch ein finales Material bereitgestellt wird.

## Revendications

1. Matériau en acier à haute teneur en manganèse, austénitique cryogénique ayant une excellente résistance à la corrosion, comprenant :
en % en poids, 0,2 à 0,5 % de C, 23 à 28 % de Mn, 0,05 à 0,5 % de Si, 0,03 % ou moins de P, 0,005 % ou moins de S, 0,001 à 0,05 % d'Al, 3 à 4 % de Cr, 0,3 à 1 % de Cu, facultativement 0,0005 à 0,01 % de B, et un reste de Fe et d'impuretés inévitables ; et
une section de concentration en Cr formée de manière continue dans une aire située à moins de 50 µm d'une surface dans une direction d'épaisseur,
dans laquelle la section de concentration en Cr inclut une section de forte concentration en Cr incluant du Cr à plus de 1,5 fois la teneur en Cr du matériau en acier et une section de faible concentration en Cr incluant du Cr à plus de 1 fois et à 1,5 fois ou moins la teneur en Cr du matériau en acier, et
dans laquelle la section de forte concentration en Cr est répartie dans une fraction de 30 % en aire ou moins, à l'exclusion de 0 %, par rapport à une superficie totale de la section de concentration en Cr,
dans lequel une limite d'élasticité du matériau en acier mesurée par un essai de propriété de traction selon la norme ASTM A370 est de 400 MPa ou plus, une résistance à la traction du matériau en acier mesurée par un essai de propriété de traction selon la norme ASTM A370 est de 800 MPa ou plus, un allongement du matériau en acier mesuré par un essai de propriété de traction selon la norme ASTM A370 est de 40 % ou plus, une résilience Charpy du matériau en acier mesurée par un essai de propriété de résilience selon la norme ASTM A370 à l'aide d'une éprouvette ayant une épaisseur d'échantillon de 10 mm est de 90 J ou plus à -196 °C, et une perte par corrosion du matériau en acier mesurée comme divulgué dans la description par un essai de résistance à la corrosion selon la norme ISO9223 de 80 mg/cm² ou moins,
et
dans lequel la fraction d'aire de la section de forte concentration en Cr est calculée en observant des portions de surface de l'éprouvette à l'aide d'un microscope électronique à balayage.

2. Matériau en acier selon la revendication 1, dans lequel la section de forte concentration en Cr est répartie dans une fraction de 10 % d'aire ou moins par rapport à une superficie totale de la section de concentration en Cr.

3. Matériau en acier selon la revendication 1, dans lequel une taille des grains d'austénite est de 5 à 150 µm.

4. Procédé de fabrication d'un matériau en acier à haute teneur en manganèse, austénitique cryogénique ayant une excellente résistance à la corrosion de la revendication 1, le procédé comprenant :
le réchauffage d'une brame incluant, en % en poids, 0,2 à 0,5 % de C, 23 à 28 % de Mn, 0,05 à 0,5 % de Si, 0,03 % ou moins de P, 0,005 % ou moins de S, 0,001 à 0,05 % d'Al, 3 à 4 % de Cr, 0,3 à 1 % de Cu, facultativement 0,0005 à 0,01 % de B, et un reste de Fe et d'impuretés inévitables, dans une plage de températures de 1050 à 1300 °C ;
le laminage à chaud de la brame réchauffée à une température de laminage de finition de 900 à 950 °C, pour obtenir ainsi un matériau intermédiaire ; et
le refroidissement du matériau intermédiaire jusqu'à une plage de températures de 600 °C ou moins à une vitesse de refroidissement de 10 à 100 °C/s, pour obtenir ainsi un matériau final.
